

No. 810,138.

PATENTED JAN. 16, 1906.

W. R. GREEN.  
ABSORBENT MATERIAL.  
APPLICATION FILED JULY 25, 1904.



Witnesses  
R. M. Cittman  
F. B. Maynard.

Inventor  
Willard R. Green  
By his Attorney  
J. H. Richards.

# UNITED STATES PATENT OFFICE.

WILLARD R. GREEN, OF MUSCATINE, IOWA.

## ABSORBENT MATERIAL.

No. 810,138.

Specification of Letters Patent.

Patented Jan. 16, 1906.

Application filed July 25, 1904. Serial No. 217,971.

*To all whom it may concern:*

Be it known that I, WILLARD R. GREEN, a citizen of the United States, residing in Muscatine, in the county of Muscatine and State 5 of Iowa, have invented certain new and useful Improvements in Absorbent Materials, of which the following is a specification.

This invention relates to absorbent materials for hygienic and surgical purposes, the 10 object being to furnish such a material adapted to be made mainly or wholly of wood that shall have an active absorptive capacity combined with efficiency in the distribution and retaining capacity of the material for the absorption and retention of fluid and semifluid 15 substances.

In the drawings accompanying and forming a part of this specification, Figure 1 is a perspective view illustrative of a mass of absorptive material made in accordance with 20 my present improvements. Fig. 2 illustrates one way of putting up or packing the material for market by making the same in the form of a sheet which is then formed into a 25 roll of a suitable size and proportions to suit the requirements of the trade. Fig. 3 is a somewhat-enlarged view of a small quantity of material for further illustrating in a somewhat 30 diagrammatic way certain features characteristic of the material.

Similar characters of reference designate like parts in all the views.

One of the principal objects of my present invention is to provide an absorbent material 35 adapted to be manufactured from materials which are abundant and of very low cost as compared with the price of cotton and flax; also, to furnish such a material of superior qualities and efficiency as an absorbent for 40 use in taking up fluid and semifluid substances; also, to furnish a material adapted to be used as a substitute for "absorbent cotton" or "absorbent linen" in many of the applications for which those materials have here- 45 tofore been employed.

When cotton or linen fibers are used in the form of an ordinary bat or unorganized mass of fiber, the tendency of the fibers is to yield almost instantly under the influence of fluids, 50 especially water, and when wetted to saturation to settle and pack more closely together, thereby forming a compact surface portion on the mass, which surface portion or layer then operates to prevent the passage of more 55 fluid into the interior of the mass. Besides having these and other well-known objec-

tions the demand for cotton and linen fiber in other arts has made the same so expensive that a much cheaper material has become commercially of exceptional importance. 60

My present improvement has as one of its objects to furnish an efficient kind of absorbent material adapted to be made chiefly or wholly of wood and adapted to be used as a substitute for absorbent cotton and 65 for other "absorbent" so-called "vegetable" fibers.

With these objects in view in the manufacture of my improved absorbent material (indicated by E, Figs. 1 and 2) I select a suitable wood or woods—such, for instance, as bass, spruce, or other suitable timber—and manufacture the same into two kinds of stock. One kind of this stock, as 16, Figs. 2 and 3, is prepared by mechanically dividing 70 or shaving a quantity of wood into strands, each of which, however finely divided it may be, is made up of many fibers and is to a large extent of a ribbon-like formation, yet preferably of such small dimensions as to 75 have a character somewhat analogous to the so-called "vegetable" fibers; but in practice the woody strands so prepared may be considerably larger and more rigid than the vegetable fiber, such as cotton or linen or wood 80 fiber, and can be more properly described as "excelsior," which may be of various grades and sizes of fineness, according to the particular purpose to which it is to be put. Another 85 portion of the wood I prepare by a cutting or grinding treatment—such, for instance, as commonly employed in the production of wood fiber for use in making "wood-pulp" for the manufacture of paper. Such a fiber stock consists of fibers that are relatively 90 quite fine and which are also of comparatively short length. This fine fiber (indicated crudely by 18) may in practice have a small amount only of some cementitious material, preferably a light sizing, incorporated 95 therewith, not enough, however, to make the mass firm or non-absorptive, and in some cases the fiber may be employed free of any component material, especially if the process of preparation has not made the same of a so- 100 called "fluffy" nature.

The two kinds of stock, strands, or fiber having been suitably prepared, I then combine suitable quantities of each kind of such stock by alternating or incorporating the 110 fiber component of the mass with the woody strands, these being in a sense dispersed and

distributed within the mass of fiber. The coarser stock or strands then essentially retains its natural woody character as compared with the fiber from which the woody 5 characteristics largely disappear in the manufacturing operations to which the wood is subjected for disintegration and separation into its ultimate fiber component. In the material when thus built up the mass of 10 coarse and more rigid woody strands contained in the absorbent material constitute a kind of interior support somewhat in the nature of a framework for containing and sustaining the mass of fiber, so that it may be 15 said there are two component masses which are so incorporated together as, practically speaking, to concurrently occupy one space. It will be evident that if the strands were organized or combined together in the manner 20 indicated and should then be used alone such a mass would, unless unduly packed, have a large proportion of its interior space consist of spaces or channels of such relatively large size as would give them a low capillary 25 or retaining power. Beside this the mass might be of too harsh and rough a nature for some of the purposes for which absorptive fibrous materials are required. By distributing among the woody strands a relatively 30 large mass or quantity of the wood fiber the relatively large interior spaces which would otherwise exist in the material are divided up by the fibers extending into and through such spaces and channels, with the result of developing 35 a higher and more active capillary and absorptive power in the mass of material considered as a whole. Thus the relatively firm and stable strands, these retaining in a large measure their original woody 40 nature, operate to keep the entire mass open and expanded, the softer and finer fiber stock being separated and kept free of undue compression, and thereby preserving in a high degree the open and porous character of 45 the absorbent mass.

In the improved absorbent material made up as herein described the material consists of two portions of wood, of which portions one of them is divided to form strands retaining 50 their woody composition—that is, retaining the gums and other materials by which the true fiber, considered strictly as such, is held together and built up into the strands of which the wood is composed. When separated 55 from the woody composition—that is, freed from the cementitious or analogous component or materials by which the ultimate wood fiber is built up into the strands ordinarily so designated—the resulting fibers 60 are of a short and very fine character. The wood fiber separated from its original woody composition forms the filling portion of the absorbent mass, the two kinds of stock being mingled together, so that the filling portion 65 of fine fiber is alternated and incorporated

with the coarser stock or woody strands. These two kinds of stock then together form and produce the capillary and fluid-retaining interstices of the mass. The larger supporting-strands of the mass, even when made 70 from wood by very finely dividing the same, naturally retain their woody composition and characteristics, since they are not divested of the composition of material by which the wood is built up from the fine and relatively 75 short fiber that constitutes its fiber component. This fiber component when so separated becomes essentially a distinctive material having quite different characteristics from its combinations as originally existing 80 in the wood.

The strands of wood naturally constitute a species of framework or open mass within and along which the wood filaments or fibers are interspersed, and the result of this mode 85 of building up the mass produces an absorbent mass of material having, in a sense, the character of a sponge, in that the mass has relatively large conduits or channels distributed therein within which the fluids may pass 90 along, as in a small stream, while scattered throughout the mass there are smaller masses intermediate and connecting the various conduits or distributing channels and which have a relative capillary action for taking up and 95 then tending to hold in place the absorbed fluids supplied thereto through the distributing conduit-spaces. Among the natural materials a sponge is peculiarly distinguished by this relation of the larger and smaller spaces, which 100 have, as between themselves, distinctly different kinds of action, the structure of the mass also being such, in the case of a sponge particularly, as it is also in my improved absorbent material, of holding the mass up nearly 105 to the normal full size notwithstanding a large amount of fluid may have been absorbed therein. In the case of the wood fiber the absorbed fluids tend to mat or felt the mass so as to make it more compact and 110 therefore less capable of receiving and holding a large amount of fluid, and this leads to what is called "sliming over," particularly in the case of fluids which are slightly viscous or tend to coagulation. With my improved 115 material, owing in part to the frame-like nature of the woody strands, the mass is not readily compacted or largely reduced in volume by the absorption of the fluid, in this important respect having a character as already pointed out analogous to the sponge. These features distinguish my present improvements in absorbent materials from all 120 those combinations of materials heretofore made up of mixtures of various kinds of fiber—such, for instance, as those in which cotton and disintegrated wood-pulp are employed, the latter being held in place by and between the layers of cotton fibers, which 125 themselves collapse on being wet. Absorb- 130

ent materials thus built up are open to the objection described of felting or matting under the action of the fluid and are particularly objectionable on account of the freedom with which they slime over, and thus become ineffective in practice.

By the use of wood for the strands of the mass I avoid the necessity of subjecting the wood to disintegrating processes and consequently save the expense of the same, besides being able to utilize the wood in a new manner in such materials, since it is in my improved material a relatively large, strong, and resistant component of the mass adapted for receiving in the interstices thereof a relatively considerable quantity of wood fiber which would not otherwise have the requisite supporting qualities nor be able when used by itself to maintain the large conduit spaces for quickly distributing relatively large quantities of fluid to the smaller capillary spaces which are distributed throughout the mass. It should be noted that one of the qualities of these capillary spaces is first

to take up the fluid and then to resist the dislodgment or discharge of the fluid therefrom, whereas the larger conduit-spaces make very slight resistance to the passage of the small stream therethrough and have relatively slight, if any, power of holding the fluid therein against the action of gravity or against the power of suction.

The absorbent material herein shown and described is for hygienic and surgical purposes in the form of bandages or otherwise, and the term "surgical purposes" in the claim is intended to cover such uses.

Having thus described my invention, I claim—

An absorbent material for surgical purposes comprising commingled excelsior and wood fiber.

Signed at Nos. 9 to 15 Murray street, New York, N. Y., this 27th day of June, 1904.

WILLARD R. GREEN.

Witnesses:

FRANCIS H. RICHARDS,  
FRED. J. DOLE.